

Patented May 3, 1927.

1,626,637

# UNITED STATES PATENT OFFICE.

WILLIAM CHARLES SPROESSER, OF BLOOMFIELD, NEW JERSEY, ASSIGNOR TO WESTINGHOUSE LAMP COMPANY, A CORPORATION OF PENNSYLVANIA.

## GETTER FOR CONTROLLING CRYSTAL GROWTH.

No Drawing.

Application filed December 6, 1922. Serial No. 605,284.

This invention relates to getters and more particularly to such containing phosphorus and a refractory oxide such as thoria.

An object of my invention is the provision of a getter suitable for use on thoriated wire or filamentary material without initial reduction of the thoria content in said wire.

Another object of my invention is the introduction of an oxide, such as thoria, into getters containing phosphorus to prevent the reduction of thoria in thoriated filamentary material, when such getters are activated after application to such material.

15 A further object of my invention is to protect the thoria in filamentary material from the initial reducing effect of phosphorus in getters, by incorporating thoria in such getter before application to the filamentary material.

20 A still further object of my invention is the provision of a getter containing thorium oxide, which oxide remaining on the filament after flashing will increase, or, at least, will not decrease the initial efficiency of the lamp and which will cause an increase in life and bump-test strength of said filament.

Other objects and advantages of the invention will be apparent from the following detailed description.

In my copending application Serial No. 519,764, filed December 3, 1921, incandescent electric lamps, and assigned to the Westinghouse Lamp Company, there is described 25 a getter adapted to be applied to filaments for incandescent electric lamps and containing a refractory oxide such as silica, alumina, or beryllium oxide. According to said application, a preferred substance was 30 silica and a satisfactory getter was prepared by mixing together the following active ingredients with approximately the following percentages by weight:—silicon oxide 40%, phosphorus 10% and cryolite 50%.

35 Although such getter has been found very effective in greatly increasing the bump-test strength of a filament after flashing, no increase in the life of the lamp was effected. Further research has resulted in the development of a getter which not only accomplishes the results obtained by the silica getter aforementioned, but causes an increase in the life of a filament to which it

has been applied. This result is accomplished without a decrease in initial efficiency of the lamp.

40 Thoria-containing getter prepared according to my invention has the property of reducing the average temperature of a filament when initially lighted. Such a getter is therefore effective in controlling the rate of crystal growth of thoriated metallic material, such as tungsten, while such material in filamentary form is being flashed. It has been shown by C. J. Smithells, Transactions Faraday Society, June 22, 1921, that the deformation of a filament which occurs during life is a function of the crystal growth. It is known that the thoria content of tungsten filamentary material retards 45 the rate of the crystal growth and thereby reduces deformation of the filament. Thoria, as well as other refractory oxides, can be reduced, to some extent, by phosphorus and other reducing agents at high temperature.

50 The greater proportion of vacuum type lamps are only flashed before being packed for shipment. Such flashing is necessary for inspection purposes and in order to 55 effect "clean up" action. If a lamp were initially lighted on designed voltage without ballast resistance before being flashed, it would very likely burn out immediately.

55 With an ordinary phosphorus-cryolite getter, the flashing operation results in greatly reduced filament strength on account of temperature gradients and excessive heating of the filament, especially the lead-in strands. With the use of a refractory oxide, 60 such as thoria, temperature gradients at flashing are almost entirely eliminated and the filament does not become overheated. This results in retardation of crystal growth, which leaves the filament stronger and less 65 liable to be broken during shipment.

70 My invention obviates a possible initial reduction of the thoria content in a filament, to which a phosphorus containing getter has been applied, by incorporating thoria 75 or its equivalent in such getter. When the getter is activated, the phosphorus will act upon the thoria incorporated therewith, which will protect the thoria content in the filament from possible reduction by the 80 phosphorus in the getter. Thoria being

highly refractory will be retained in part, at least, on the filament and will serve to increase the strength thereof.

My invention is especially adapted for a phosphorus containing getter. It has been customary to use a getter, called 31-13, containing 100 parts, by weight, of cryolite and 13 parts, by weight, of phosphorus and I have found that such a getter is very favorably modified by replacing from 20 to 25 parts of the cryolite content by the same amount, by weight, of thoria. It has been found from the results of a large number of tests, that lamps made with thoria getters equal in bump-test strength after the flashing treatment, the lamps made with a silica getter and at the same time an improvement in life is effected, as compared with the life of such a lamp when using the ordinary phosphorus-cryolite getter.

In regard to bump-test strength, the results show that the increase varies up to over 100%, with 50% representing about the average increase. From life testing lamps using a thoria getter indicated that as an average, a 15% increase in life may be expected with the use of such getters.

The advantages of using thoria as a component of a getter material are as follows. Thoria, being inert with respect to tungsten, will not cause any deleterious reaction therewith. Any thoria remaining on the filament after flashing, will not reduce the initial efficiency of the lamp, in fact, incandescent thoria having a higher selective light emission than tungsten, should cause improvement in luminosity. Further, if as is believed by a few authorities, part of the thoria of a thoriated filament is reduced by phosphorus introduced with the getter, when the getter is activated, the use of thoria getters should materially decrease such reaction by providing additional thoria for the phosphorus to react with, instead of with the thoria content of the filament.

To explain the increase in filament strength effected by the use of thoria getters, the same reasons can be given as those used to explain that action with the use of silica getters. It is thought that one of the chief reasons for the increase in filament strength when refractory substances are used, is that of reducing temperature gradients to a minimum, particularly at the flashing operation.

Desirable results have been obtained by using thoria which was heated to a temperature of 2000° C. before being incorporated with the other materials of the getter. The heating may be done in a carbon resistance furnace using a carborundum vessel as a container. Results in some early tests, where the clean-ups after flashing were not satisfactory, indicated that the thoria contained traces of occluded gases. Heating to the

aforementioned high temperature was done to remove such gases and when such was done, satisfactory results were obtained.

As a substitute for thoria, Welsbach mixture has been tried, that is, thoria containing an admixture of 1% of ceria. Although it would appear that such a mixture would effect the same result as thoria, it has not proven to be entirely satisfactory, as the ceria appears to interact with the tungsten of the filament.

It will therefore be apparent that it is desirable to use very pure thoria, which should be thoroughly incorporated with the other materials of the getter, for example, red phosphorus and cryolite. A preferred formula for a getter according to my invention is approximately 20 to 25 parts, by weight, of thoria, 13 parts, by weight, of phosphorus and from 80 to 75 parts, by weight, of cryolite, although the proportions may be varied. For example, satisfactory results have been obtained when using up to 50 parts of thoria, with as little as 50 parts of cryolite and about 13 parts of phosphorus. A homogeneous mixture may be made of these substances and a thin coating thereof applied in any desired manner to the filamentary material. The coating may be dried and thereafter the coated filament severed into appropriate lengths and mounted in an incandescent electric lamp envelope in the usual method.

The following table shows the life test results of lamps made with the usual phosphorus-cryolite or 31-13 getter, as compared to those made with such a getter in which part of the cryolite has been replaced by thoria. In the first test only, the initial lumens is expressed as candle power.

| Test No. | Type lamp watts. | Getter composition.                           | Life test results. |                        | Life based on initial efficiency hours. | Life based on mean efficiency hours. |
|----------|------------------|-----------------------------------------------|--------------------|------------------------|-----------------------------------------|--------------------------------------|
|          |                  |                                               | Initial lumens.    | Per cent lumens maint. |                                         |                                      |
| 1....    | 40               | 20 g. ThO <sub>2</sub> , 80 g. cry., 13 g. P. | 42.2 CP.           | 89.7                   | 1677                                    | 1735                                 |
| 1....    | 40               | 31-13 (100 g. cry., 13 g. P.)                 | 42.1 CP.           | 87.5                   | 1513                                    | 1385                                 |
| 2....    | 40               | 25 g. ThO <sub>2</sub> , 75 g. cry., 13 g. P. | 404                | 87.0                   | 1099                                    | 1176 115                             |
| 2....    | 40               | 50 g. ThO <sub>2</sub> , 50 g. cry., 13 g. P. | 406                | 84.1                   | 1225                                    | 1101                                 |
| 2....    | 40               | 31-13                                         | 406                | 86.0                   | 962                                     | 1023                                 |
| 3....    | 60               | 25 g. ThO <sub>2</sub> , 75 g. cry., 13 g. P. | 632                | 78.2                   | 2080                                    | 1845                                 |
| 3....    | 60               | 31-13                                         | 619                | 80.1                   | 1564                                    | 1623                                 |
| 4....    | 40               | 25 g. ThO <sub>2</sub> , 75 g. cry., 13 g. P. | 400                | 86.4                   | 1845                                    | 2061 120                             |
| 4....    | 40               | 50 g. ThO <sub>2</sub> , 50 g. cry., 13 g. P. | 393                | 88.1                   | 1420                                    | 1865                                 |
| 4....    | 40               | 25 g. ThO <sub>2</sub> , 75 g. cry., 13 g. P. | 398                | 85.1                   | 1279                                    | 1430                                 |
| 4....    | 40               | 31-13                                         | 393                | 88.9                   | 764                                     | 991                                  |
| 5....    | 40               | 25 g. ThO <sub>2</sub> , 75 g. cry., 13 g. P. | 396                | 89.8                   | 1034                                    | 1388                                 |
| 5....    | 40               | 50 g. ThO <sub>2</sub> , 50 g. cry., 13 g. P. | 406                | 88.0                   | 1078                                    | 1223 125                             |
| 5....    | 40               | 31-13                                         | 401                | 84.4                   | 1554                                    | 1516                                 |
| 5....    | 40               | 31-13                                         | 396                | 91.7                   | 800                                     | 1290                                 |

Although I have described what is now considered the preferred embodiment of my

invention it is to be understood that modifications may be made therein within the spirit and scope of the appended claims.

What is claimed is:

5. 1. A getter for application to a thoriated tungsten filament for an incandescent electric lamp comprising thoria for increasing the life and bump-test strength of said filament.
- 10 2. A getter for application to a thoriated tungsten filament of an incandescent electric lamp comprising thoria and phosphorus, the thoria serving to prevent initial reduction of the thoria in the filament by the phosphorus during flashing, whereby the crystal growth restraining effect of the filament contained thoria is maintained.
- 15 3. A getter for a thoriated tungsten filament prepared according to approximately the following proportions: 20 to 25 parts by weight of thoria, about 13 parts by weight of phosphorus and 80 to 75 parts by weight of cryolite.

4. In an incandescent electric lamp, a thoriated tungsten filament having a coating 25 of a thoria-containing getter, whereby excess crystal growth in the filament is prevented.

5. In an incandescent electric lamp, a thoriated tungsten filament coated with a 30 getter comprising thoria and phosphorus, whereby excessive crystal growth in the filament is prevented.

6. In an incandescent electric lamp, a thoriated tungsten filament having applied 35 thereto, a getter prepared according to approximately the following proportions: 20 to 25 parts by weight of thoria, about 13 parts by weight of phosphorus and 80 to 75 parts by weight of cryolite, the thoria serving to 40 prevent excessive crystal growth in the filament.

In testimony whereof, I have hereunto subscribed my name this 5th day of December, 1922.

WILLIAM CHARLES SPROESSER.